

## UNITED STATES PATENT OFFICE

2,578,851

## LUBRICATING GREASES

Herschel G. Smith, Wallingford, Troy L. Cantrell, Lansdowne, and Mark L. Hill, Boothwyn, Pa., assignors to Gulf Oil Corporation, Pittsburgh, Pa., a corporation of Pennsylvania

No Drawing. Application September 12, 1949,  
Serial No. 115,314

8 Claims. (Cl. 252—33.6)

1

This invention relates to novel lubricating greases and, more particularly, to soap-thickened mineral oils having a modified gel structure.

Difficulties have been encountered in the use of conventional mineral oil greases because of the fact that these conventional greases sometimes have indefinite and unstable gel structure. Slight variations in soaps or other basic ingredients produce changes in the gel structure which result in oil separation and limit the efficiency of the grease, its service life and the uses to which it can be applied.

It is therefore an object of this invention to produce a soap-thickened grease which has a modified gel structure.

Another object of this invention is to manufacture a grease in which oil separation or bleeding does not take place.

A further object of this invention is to provide a grease which can be used on high pressure bearings.

These objects are accomplished in accordance with the present invention by the preparation of a grease which comprises a major amount of a mineral oil thickened to a grease with a soap and a minor amount, sufficient to prevent bleeding, of a metal phthalyl alkyl amide (a metal salt of an N-alkyl phthalimidic acid) having the generic formula



wherein M is a metal, x is a whole number equal to the valence of M, and R is an alkyl group containing from 8 to 20 carbon atoms.

In a soap-thickened mineral oil type of grease, the soaps generally employed as thickeners include the sodium, calcium, aluminum and zinc or other metal salts of fatty materials derived from animal or vegetable fats or fatty acids. For example, the metal of the soap can be an alkali metal, an alkaline earth metal, and various other metals such as lead, chromium, tin, iron, cobalt, nickel, cadmium, mercury, etc., and the fats or fatty acids can be tallow, lard, cotton-seed oil, stearic acid, soy bean fatty acids and various other fats or fatty acids. The mineral oil employed is an appropriate grade of lubricating oil of naphthenic, paraffinic or mixed base with a viscosity suitable for the proposed function. These greases themselves are well known in the art and can be manufactured by conventional methods. As will be understood by those skilled in the art, the soap and mineral oil base will be selected in accordance with the specific properties of the grease it is desired to manu-

2

facture. Our invention therefore contemplates the addition of a metal phthalyl alkyl amide to any grease comprising a mineral oil thickened to the consistency of a grease with a soap. By the term "soap-oil grease" or "soap-thickened grease", we refer to these commonly known greases.

In the preparation of the greases of our invention the soap-oil greases are usually prepared first, and subsequently, from 0.1 to 5.0 per cent by weight on the grease of the metal phthalyl alkyl amide is incorporated in the grease. However, the metal phthalyl alkyl amide may be added during the manufacture of the grease, for example, by being dissolved in the mineral oil used in compounding the grease.

The nature of our lubricating grease composition will be more clearly understood by reference to the following examples.

## EXAMPLE I

A grease having the following composition was prepared by the conventional pressure saponification method:

|                                                |         |     |
|------------------------------------------------|---------|-----|
| 25. No. 1 lard oil                             | gallons | 150 |
| Water                                          | do      | 14  |
| 150 pale coastal oil (156 S. U. S. at 100° F.) | gallons | 900 |
| Powdered hydrated lime                         | pounds  | 198 |
| 30. No. 1 inedible tallow                      | do      | 100 |

The lubricant was then dehydrated and, during the stirring and cooling operation, 1 per cent by weight of the calcium salt of N-dodecylphthalimidic acid was added.

## EXAMPLE II

A cup grease having the following composition in parts by weight was prepared by the pressure saponification method:

|                                              |      |
|----------------------------------------------|------|
| 40. Red engine oil (205 S. U. S. at 100° F.) | 83.2 |
| Calcium soap of tallow                       | 14.4 |
| Glycerin                                     | 1.4  |
| Water                                        | 1.0  |

45 During the stirring and cooling operation, 1 per cent by weight of the calcium salt of N-dodecylphthalimidic acid was incorporated therein.

## EXAMPLE III

A recoil mechanism grease having the following composition in parts by weight was prepared by the pressure saponification method:

|                                         |    |
|-----------------------------------------|----|
| 55. Texas oil (500 S. U. S. at 100° F.) | 17 |
| Texas oil (1900 S. U. S. at 100° F.)    | 62 |
| Aluminum stearate                       | 17 |

Two per cent by weight of the aluminum salt of N-dodecylphthalimidic acid was subsequently 60 incorporated therein.

## EXAMPLE IV

A roller bearing grease was prepared having the following composition:

|                                         | Per cent by weight |
|-----------------------------------------|--------------------|
| Sodium tallow soap                      | 14                 |
| 400 S. U. S. lubricating oil at 100° F. | 86                 |

The above grease was treated with 1 per cent by weight of the sodium salt of N-hexadecylphthalimide acid.

The viscosities expressed for the oils in the above examples are in Saybolt Universal seconds at 100° F. It is obvious that any of the soap-oil greases can be used in accordance with our invention and that the above examples are merely illustrative. Variations will naturally occur to those skilled in the art.

The metal phthalyl alkyl amides which are incorporated in the soap-oil greases in accordance with this invention are readily prepared, as will be shown, from metal hydroxides, phthalic anhydride and primary alkyl amines; or, in the event the metal hydroxide of a particular metal is difficult to react, as, for example, the heavy metal hydroxides, the desired heavy metal N-alkyl phthalimide can be readily prepared by first preparing an alkali metal N-alkyl phthalimide and reacting the latter with a water soluble salt of the desired heavy metal by a conventional double decomposition or metathesis reaction. We obtain particularly good results from the sodium, calcium and aluminum N-alkyl phthalimides; however, satisfactory metal salts of N-alkyl phthalimides can be prepared from potassium, or other alkali metal, barium, strontium, magnesium, chromium, nickel, cobalt, zinc, lead, tin, copper, cadmium, bismuth, etc.

The primary alkyl amines which we employ in the preparation of the metal phthalyl alkyl amides are amines having the following generic formula:



wherein  $n$  is a number between 6 and 18. Some 45 of the amines of this generic class are

Mono-capryl amine

Mono-lauryl amine

Mono-myristyl amine

Mono-palmityl amine

Mono-stearyl amine

and other primary alkyl amines having the above formula. Any of the above amines may be used with advantage in making our metal phthalyl alkyl amides. Furthermore, mixtures of such amines may be employed. For instance, one commercially available mixture of such amines is the so-called "cocoamine" prepared by converting the mixed acids of coconut oil into corresponding amines by well known methods. The commercial "cocoamine" has an average molecular weight of about 200-210 and contains a major amount of dodecylamine.

In preparing our metal phthalyl alkyl amides, we usually react the primary alkyl amine with phthalic anhydride in substantially equimolecular amounts to form a mono-alkyl amide of phthalic acid, and then neutralize the residual acidity of that compound by reaction with the desired metal hydroxide, sufficient metal hydroxide being employed to form substantially neutral metal salts thereof. These reactions can be advantageously effected in the presence of sufficient mineral oil to dissolve the oil-soluble com-

5 pounds so obtained, the new improvement agents being formed in situ in the oil.

The following examples illustrate various methods of preparing our metal phthalyl alkyl amides.

## EXAMPLE A

In this example, the improvement agent was prepared in situ in mineral oil from phthalic anhydride, dodecylamine and aluminum hydroxide, the agent so prepared having the following formula:



The procedure employed in preparing this compound was as follows:

25 Into an iron vessel equipped with means for heating, stirring and cooling, were charged 444 pounds of phthalic anhydride to which 555 pounds of dodecylamine were slowly added. To this mixture were added 2000 pounds of a Texas oil having a viscosity of 70 S. U. S. at 100° F. and the components were thoroughly agitated and slowly heated to 120° F. After one hour, 435 pounds of alumina (gelatinous 18 per cent  $\text{Al}(\text{OH})_3$ ) were added and the mixture was kept 30 at 140° F. until the formation of water was completed and no more water could be drawn off.

35 From the kettle 2966 pounds of aluminum phthalyl dodecyl amide oil mixture were obtained.

40 The aluminum phthalyl dodecyl amide produced in situ in oil had the following properties:

Gravity, °API

20.8

Viscosity, SUV:

100° F. 295

210° F. 61.5

Neutralization No. 1.11

## EXAMPLE B

50 A calcium phthalyl alkyl amide having the following formula:



60 where R is an octadecyl radical, was prepared from 74 grams of phthalic anhydride, 135 grams of mono-octadecylamine, 19 grams of hydrated lime and 400 grams of mineral oil. In preparing this agent, the phthalic anhydride and amine were heated together in the oil until dissolved therein. Then the dry lime was added, whereupon a violent reaction occurred. After this vigorous reaction subsided, the mixture was heated to 400° F. to complete the reaction and remove the water formed as a by-product of these reactions. The so dehydrated material, while still hot and fluid, was filtered to remove any insoluble matter. The substantially anhydrous oil solution of the calcium N-mono-octadecyl amido phthalate compounds so obtained was then cooled to room temperature.

70 The metal phthalyl alkyl amides which are de-

scribed in the above examples have been used as additives in mineral lubricating oils because of the antirust and anticorrosion properties which they confer upon the lubricants in which they are incorporated. The calcium and aluminum salts of phthalamic acid are described in U. S. Letters Patent Nos. 2,378,442 and 2,378,443. It is true that, as in the case of mineral oils, metal phthalyl alkyl amides also render grease compositions non-corrosive to metal parts. Our invention, however, resides in the discovery that entirely new and unexpected results are obtained by the addition of metal phthalyl alkyl amides to soap-oil greases. ~~...to the claims~~ We have discovered that the metal phthalyl alkyl amides modify the gel structure of the grease. Due to the fact that the grease has a different gel structure, the following properties of the grease are improved:

(1) The new gel structure does not break down as readily as the gel structure in the unmodified grease.

(2) A more plastic grease is produced.

(3) The texture of the grease is smoother and more uniform.

(4) The gel is notably stabilized against bleeding and oil evaporation.

Moreover, the grease does not become rancid over a long storage period because the metal phthalyl alkyl amide acts as a buffer to the soap solution.

The grease compositions of our invention have all been rigidly tested according to the methods prescribed in Army-Navy Aeronautical Specifications for Grease, AN-G-3a for lubricating performance, life, bleeding, evaporation, apparent viscosity, plasticity and low temperature torque. These tests clearly establish the fact that the gel structure of the original grease has been modified. The following comparative tests show the amount of bleeding and evaporation according to the Army-Navy standard specification tests.

#### Bleeding and evaporation test

##### TEST AN-G-3a

| Grease                                                                                                            | Per cent of separated oil due to bleeding and evaporation after 50 hours (212° F.) |
|-------------------------------------------------------------------------------------------------------------------|------------------------------------------------------------------------------------|
| Grease prepared according to Example I and modified with 1% of calcium N-dodecyl phthalamate.                     | 0                                                                                  |
| Grease prepared according to Example I but not modified.                                                          | 24                                                                                 |
| Cup grease prepared according to Example II and modified with 1% of calcium N-dodecyl phthalamate.                | 0                                                                                  |
| Cup grease prepared according to Example II but not modified.                                                     | 28                                                                                 |
| Recoil mechanism grease prepared according to Example III and modified with 2% of aluminum N-dodecyl phthalamate. | 0.1                                                                                |
| Recoil mechanism grease prepared according to Example III but not modified.                                       | 12                                                                                 |
| Roller bearing grease prepared according to Example IV and modified with 1.0% of sodium N-hexadecyl phthalamate.  | 0                                                                                  |
| Roller bearing grease prepared according to Example IV but not modified.                                          | 5                                                                                  |

The above tests clearly indicate the stability of our greases against bleeding or separation, particularly since our greases showed no signs of bleeding during the fifty-four hour test period. In fact, the unmodified greases showed some bleeding within 48 hours while the modified grease was still without separation after a two-week period.

The greases prepared according to our inven-

tion give eminently satisfactory lubrication, especially when used on high pressure bearings at high surface temperatures. These greases are not consumed at an excessive rate while they are lubricating such hot bearings. In all cases the compositions give satisfactory lubrication in such applications as gun mechanisms, roller bearings and similar mechanisms.

Resort may be had to such modifications and variations as fall within the spirit of the invention and the scope of the appended claims.

#### We claim:

1. A lubricating grease which comprises a major amount of a soap-oil grease, and a minor amount, sufficient to prevent bleeding, of a metal phthalyl alkyl amide having the formula



wherein R is an alkyl group containing from 8 to 20 carbon atoms, X is a whole number equal to the valence of M, and M is a metal.

2. A lubricating grease having a modified gel structure, comprising a major amount of a soap-oil grease and a minor amount, from 0.1 to 5.0 per cent by weight of said soap-oil grease of a metal phthalyl alkyl amide having the formula



wherein R is an alkyl group containing from 8 to 20 carbon atoms, X is a whole number equal to the valence of M, and M is a metal.

3. A lubricating grease having a modified gel structure which comprises a major amount of a soap-oil grease and a minor amount, sufficient to prevent bleeding, of a sodium phthalyl alkyl amide having the formula



wherein R is an alkyl group containing from 8 to 20 carbon atoms.

4. The grease of claim 3 wherein R is a hexadecyl radical.

5. A lubricating grease having a modified gel structure which comprises a major amount of a soap-oil grease and a minor amount, sufficient to prevent bleeding, of a calcium phthalyl alkyl amide having the formula



wherein R is an alkyl group containing from 8 to 20 carbon atoms.

6. The grease of claim 5 wherein R is a dodecyl radical.

7. A lubricating grease having a modified gel structure which comprises a major amount of a soap-oil grease and a minor amount, sufficient to

prevent bleeding, of an aluminum phthalyl alkyl amide having the formula



wherein R is an alkyl group containing from 8 to 15 20 carbon atoms.

8. The grease of claim 7 wherein R is a dodecyl radical.

HERSCHEL G. SMITH,  
TROY L. CANTRELL,  
MARK L. HILL.

## REFERENCES CITED

The following references are of record in the file of this patent:

## UNITED STATES PATENTS

| Number    | Name               | Date           |
|-----------|--------------------|----------------|
| 2,378,442 | Smith et al. ----- | June 19, 1945  |
| 2,378,443 | Smith et al. ----- | June 19, 1945  |
| 2,408,102 | Smith et al. ----- | Sept. 24, 1946 |
| 2,408,103 | Smith et al. ----- | Sept. 24, 1946 |